

# UNITED STATES PATENT OFFICE.

RICHARD JESCHKE, OF CHARLOTTENBURG, GERMANY, ASSIGNOR TO PHENOLEUM  
G. M. B. H., OF BERLIN, GERMANY, A FIRM.

## FLOORING MATERIAL AND PROCESS FOR MAKING SAME.

1,421,036.

Specification of Letters Patent. Patented June 27, 1922.

No Drawing.

Application filed July 9, 1920. Serial No. 395,181.

To all whom it may concern:

Be it known that I, RICHARD JESCHKE, a citizen of the German Empire, and resident of Charlottenburg, in the State of Prussia, German Empire, have invented new and useful Improvements in Flooring Materials and Processes for Making Same, of which the following is a full, clear, and exact specification.

10 My invention relates to materials suitable for covering floors and the like and similar to the well-known linoleum and to the process of preparing such material.

15 My new product is distinguished from those hitherto used by the fact that neither oxidized linseed oil nor any other oils are used in its manufacture. By dispensing with these starting materials, which are expensive and sometimes difficultly available, 20 I realize a remarkable economy when compared with the usual products. Further, my product has the advantage that it is immediately ready for use and does not want as linoleum does, storing for a rather long period and drying, time, storing rooms and drying appliances being thus dispensed with. 25 My new product is very tough and flexible or elastic, so that it is not necessary to apply it to a lining of textile fabrics, paper or the like as is necessary in the case of linoleum. However, if desired, such a lining can of course be used.

According to my invention I first prepare two ingredients, viz: (1) the rubber-like product obtained by heating glue or other glutinous substances or carbon hydrates with glycerin and (2) artificial resins prepared by acting upon phenols and formaldehyde with alkaline condensing agents, such as caustic alkalis or alkali carbonates. I then mix these ingredients and heat the mixture until a tough mass is formed. While heating, a certain quantity of formaldehyde that has not entered the reaction, acts as a 45 hardening agent. Other hardening agents such as chromium salts, alum, tannin or the like may be added if desired, care being taken however in all cases to ensure a sufficient elasticity of the product.

50 The product thus obtained can then be treated in the manner known in connection with linoleum by mixing it with cork meal and kneading and rolling the mixture in the manner well known to those skilled in the art. For cork meal I can substitute partly

or wholly other filling agents, such as wood meal or other finely disintegrated cellulose. If it is desired to obtain a coloured product, pigments may be added to the mixture. If desired, the mass can be rolled upon a lining 60 of paper or textile fabric but, as already mentioned, such lining is not absolutely necessary.

For the glycerin used in preparing the first ingredient above referred to, other substances which are hygroscopic or prevent the mixture from drying may be substituted such substances being for instance potassium sulfocyanate which may be used as an aqueous solution.

70 In practically carrying out my process I can for instance proceed as follows:

Example: I first prepare the two ingredients of the mixture. 200 grammes of glue or gelatine are allowed to swell in water and 75 heated with 450 grammes of glycerin for about 15 minutes up to about 90° C.

On the other hand, 300 grammes of phenol or crystallized carbolic acid are heated with 300 grammes of a 35 per cent formaldehyde 80 solution and 50 grammes of potassium carbonate or the corresponding quantity of sodium carbonate or caustic soda solution for about 10 minutes up to about 100° C.

The artificial resin thus obtained is mixed 85 with equal parts of the mass obtained from glue and glycerin and the mixture is heated until a tough viscous mass is obtained. During this heating a certain quantity of formaldehyde that has not entered the reaction, 90 acts to harden the product.

Instead of carbolic acid other phenols, creosote or the like may be used.

I then take 18 parts by weight of the mass so obtained and I mix them with 18 parts 95 of cork meal or wood meal and if desired with 12 parts of a pulverized pigment. The pastous mass thus obtained is then kneaded and rolled in the well-known manner.

The proportions indicated may be modified according to the requirements of the special case and to the properties desired of the product to be obtained.

Having thus described my invention I wish it to be understood that I do not desire to limit myself to the exact details and proportions given, as obvious modifications will occur to persons skilled in the art.

What I claim is:—

1. The process of manufacturing linoleum- 110

like material, which process consists in mixing the following two ingredients, viz the product obtained by heating glycerin with an organic compound, capable of forming a 5 rubber-like product by acting on glycerin, for producing therewith a rubber like product, and an artificial resin obtained by condensing a phenol with formaldehyde by means of an alkaline condensing agent, heating 10 the mixture until a tough mass is formed, adding a filling agent, and kneading and rolling the mixture thus obtained.

2. The process of manufacturing linoleum-like material, which process consists in mixing 15 the following two ingredients, viz the product obtained by heating glycerin with an organic compound, capable of forming a rubber-like product by acting on glycerin, for producing therewith a rubber like product, and an artificial resin obtained by condensing a phenol with formaldehyde by means of an alkaline condensing agent, heating the mixture until a tough mass is formed, adding a hardening agent during the last 20 part of the heating process, then adding a filling agent, and kneading and rolling the mixture thus obtained.

3. The process of manufacturing linoleum-like material, which process consists in mixing 30 the following two ingredients, viz the product obtained by heating glycerin with a glutinous substance, and an artificial resin obtained by condensing a phenol with formaldehyde by means of an alkaline condensing agent, heating the mixture until a tough mass is formed, adding a filling agent, and kneading and rolling the mixture thus obtained.

4. The process of manufacturing linoleum-like material, which process consists in mixing 40 the following two ingredients, viz the product obtained by heating glycerin with a glutinous substance, and an artificial resin obtained by condensing a phenol with formaldehyde by means of an alkaline condensing agent, heating the mixture until a tough mass is formed, adding a hardening agent during the last part of the heating process, then adding a filling agent, and kneading 45 and rolling the mixture thus obtained.

5. The process of manufacturing linoleum-like material, which process consists in mixing equal parts by weight of the following two ingredients, viz the product obtained 55 by allowing 200 grammes of gelatine to swell in water and heating them with 450 grammes

of glycerin up to about 90° C. for about 15 minutes, and the artificial resin obtained by heating 300 grammes of phenol with 300 grammes of a 35 per cent formaldehyde solution and 50 grammes of potassium carbonate up to about 100° C. for about 10 minutes, heating the mixture of these two ingredients until a tough viscous mass is formed, mixing 18 parts by weight of this 60 mass with about 18 parts by weight of cork meal and about 12 parts by weight of a pulverized pigment and kneading and rolling the mixture thus obtained.

6. The herein described linoleum-like composition consisting of a mixture of 200 grammes of gelatine with 450 grammes of glycerin and an artificial resin prepared from 300 grammes of phenol and 300 grammes of a 35 per cent formaldehyde solution and 50 grammes of potassium carbonate with an equal weight of cork meal.

7. The herein described linoleum-like composition consisting of a mixture of 200 grammes of gelatine with 450 grammes of glycerin and an artificial resin prepared from 300 grammes of phenol and 300 grammes of a 35 per cent formaldehyde solution and 50 grammes potassium carbonate with an equal weight of cork meal and approximately two-thirds of its weight of a pulverized pigment.

8. The herein described linoleum-like composition consisting essentially of a mixture of a filling agent, a rubber like product obtained from glycerin and an artificial resin obtained from a phenol.

9. The process of manufacturing linoleum-like material, which process consists in mixing the following two ingredients, viz the product obtained by heating glycerin with an organic compound, capable of forming a rubber-like product by acting on glycerin, for producing therewith a rubber-like product, and an artificial resin obtained by condensing a phenol with formaldehyde by means of an alkaline condensing agent, heating the mixture until a tough mass is formed, adding a filling agent, and kneading and rolling the mixture thus obtained.

In testimony, that I claim the foregoing as my invention, I have signed my name in presence of two subscribing witnesses.

RICHARD JESCHKE.

Witnesses:

RUDOLPH KOMICKE,  
WILHELM STRAUSS.